

(No Model.)

F. SEDGWICK.

PROCESS OF MANUFACTURING STEEL COATED WIRE.

No. 443,464.

Patented Dec. 23, 1890.

Fig. 1.



Fig. 2.



Witnesses:

Law. S. Curtis.

Mary M. Farr

Inventor:

Frederick Sedgwick

By Murray Evans & Clark  
Attorneys.

# UNITED STATES PATENT OFFICE.

FREDERICK SEDGWICK, OF CHICAGO, ILLINOIS, ASSIGNOR TO THE AMERICAN SPRING COMPANY, OF ILLINOIS.

## PROCESS OF MANUFACTURING STEEL-COATED WIRE.

SPECIFICATION forming part of Letters Patent No. 443,464, dated December 23, 1890.

Application filed May 11, 1888, Serial No. 273,602. (No specimens.)

*To all whom it may concern:*

Be it known that I, FREDERICK SEDGWICK, a citizen of the United States, residing in Chicago, in the county of Cook and State of Illinois, have invented a new and useful Improvement in the Process of Manufacturing Steel-Coated Wire, of which the following is a specification.

The object of this invention is the production of steel-coated wire.

It is well understood that in order to successfully convert the surface of iron into steel for the purpose of case-hardening it or otherwise the metal treated, when immersed in the material or bath by which its surface is converted into steel, must not only retain its heat a sufficient length of time to enable the steelifying compound or mixture to do its work, but must also maintain a sufficiently high temperature to insure the active operation of the compound or mixture. This feature of the process has heretofore prevented its use with small bodies of iron, because of their inability to maintain the heat at the proper degree or for the requisite time. In the case of continuous or "long" wire the length has also formed an obstacle to its being case-hardened. In this invention I overcome these obstacles as follows: I subject the wire to the heating action of electricity while it is immersed in the steelifying material or bath by connecting it at either side of the bath with the poles of a battery, dynamo, or other generator of electricity, so that the wire shall complete an electrical circuit and be heated by the current from the generator. In this manner I insure the presence in the wire of the requisite amount of heat during the entire time it remains in the bath. To harden

the casing of the wire thus converted into steel, it is only necessary to chill the wire quickly, and this may be done by putting it into a chilling-bath as soon as the steelifying operation is over. In the case of the continuous or long wire this is conveniently done by drawing the wire directly from the steelifying bath or receptacle into a chilling-bath.

In the accompanying drawings I have shown a form of apparatus specially designed for the working of my process in the case of

long or continuous wire, and which I believe to be the best form of apparatus for the purpose, Figure 1 being a side elevation of the apparatus, and Fig. 2 a longitudinal section thereof.

In said drawings, A A' represent spools located at either end of the apparatus, the former containing the wire to be treated and the latter being intended to receive it after the operation. Spool A' may be driven by the belt *a* and pulley *a'*, and thus draw the wire from spool A by a continuous or intermittent movement. Intermediate said spools are the vats or receptacles B and C, and the wire (indicated by *W*) passes through both these, receiving in the first one its bath or charge of steelifying chemicals or material, and in the second a chilling-bath. Into vat B, I put any of the known compounds or mixtures used in case-hardening operations, such as ferrocyanide of potash, and the wire comes in contact therewith while *en route* through vat B and takes up such a charge thereof as the time consumed in the passage through the vat and the degree of heat present in the wire will permit, both time and temperature being entirely under the control of the operator. The vat C is located closely adjacent to vat B, so the wire may not become cool in its travel from one vat to the other. Vat C is preferably supplied with metallic shot, particles of metal, or equivalent small-sized material *c*, which act upon the wire as it passes and free it of all bubbles, roughness, and adhering material, and such shot may be supported in a wire basket *D*, thereby giving the cooling-fluid supplied by the pipe *E* freedom to reach the inclined floor *d* of the vat, and thus gain access to the drain *e*.

While in vat B the wire is heated to the requisite red heat by electricity conducted to it from the dynamo or other source of electric energy *F*, the wire *G* carrying the current from one pole of the dynamo to the post *g*, with which the wire *W* is in constant contact, and the wire *H* carrying the current from the other pole of the dynamo into the body of shot in vat C, so that that portion of the wire under treatment which extends from post *g* to the shot in vat C completes the

electric circuit, and thus receives any necessary amount of heat from the dynamo. The electric wire H may connect with wire W shortly in advance of the chilling-vat, if thought more desirable. After being thus heated in the presence of the steel-converting material or chemical the wire may be then chilled in vat C or in any known way, so as to harden the coating of the wire. Of course, if the hardening feature should not be desired, the chilling-vat should be omitted from the apparatus, and if short lengths or bodies of metal are operated upon the spools are unnecessary.

15 In order that no portion of the electric fluid shall be diverted from the wire W, I insulate the latter from vat B, unless said vat is made of non-conducting material, by means of the asbestos *i*, at the openings through which the wire passes. A like insulating plug *i'* may be used at the initial end of the vat C.

Where the converting material is in fluid form it may be advisable to separate the two vats somewhat in order to give the coating of the fluid which would then adhere to the wire a little time to harden before it enters the chilling-vat, and this feature may perhaps prove advisable with other kinds of steelify-

ing material. So, too, the wire may be depressed below the plane of the wire openings in vat B by rollers or otherwise, if that is desirable, to prevent leakage at such openings.

It will be understood that I do not limit myself in the matter of the carbonizing material, nor to the construction of vat for administering it to the wire, because any material known to be adapted to effect the carbonizing or steelifying result, whether in solid, powder, fluid, or gaseous form, may be employed, and the vat, which is only the instrument whereby the carbonizing material, fluid, or gas is brought into contact with the wire, may be changed to suit the nature of the carbonizing agent.

I claim—

The process of converting the surface of wire into steel, consisting in drawing the wire through a steelifying bath or material and heating that portion of the wire which is in the act of passing through the bath or material by means of an electric current, substantially as set forth.

FREDERICK SEDGWICK.

Witnesses:

EDW. S. EVARTS,

EDMUND ADCOCK.